

# United States Patent [19]

Aoki et al.

[11] Patent Number: 4,674,592

[45] Date of Patent: Jun. 23, 1987

[54] DIAPHRAGM FOR USE IN  
ELECTRO-ACOUSTIC TRANSDUCER

[75] Inventors: **Shuichi Aoki**, Tokyo; **Katsuyoshi Kumagai**, Yamagata; **Akihiko Haga**, Yamagata; **Minoru Ito**, Yamagata, all of Japan

[73] Assignee: **Alpine Electronics Inc.**, Tokyo, Japan

[21] Appl. No.: 796,896

[22] Filed: Nov. 12, 1985

## [30] Foreign Application Priority Data

Nov. 14, 1984 [JP] Japan ..... 59-238566

[51] Int. Cl.<sup>4</sup> ..... G10K 13/00

[52] U.S. Cl. ..... 181/170; 428/64;  
428/341; 428/342; 428/476.3; 428/479.3;  
428/479.6

[58] Field of Search ..... 181/157, 167, 169, 170;  
428/64, 341, 342, 476.3, 479.3, 479.6

[56]

## References Cited

### U.S. PATENT DOCUMENTS

2,006,830 7/1935 Howley ..... 181/169  
4,076,098 2/1978 Wood ..... 181/170

### FOREIGN PATENT DOCUMENTS

0071619 6/1979 Japan ..... 181/170

Primary Examiner—Benjamin R. Fuller  
Attorney, Agent, or Firm—Murray and Whisenhunt

[57]

## ABSTRACT

A diaphragm for use in an electro-acoustic transducer comprises a diaphragm main body only or mainly composed of natural fibers, a layer formed by laminating thereover a polyamide resin and a synthetic resin coating layer further formed to the surface of the laminate layer. The diaphragm is free from pin holes, exhibits satisfactory water proofness and excellent physical properties such as sonic propagation velocity inherent to the natural fibers. It can be fabricated with ease at a good yield and can reduce the fabrication cost.

1 Claim, 5 Drawing Figures



FIG. 1



FIG. 2



FIG. 3



FIG. 4



FIG. 5



## DIAPHRAGM FOR USE IN ELECTRO-ACOUSTIC TRANSDUCER

### BACKGROUND OF THE INVENTION

This invention relates to a diaphragm for use in electro-acoustic transducer such as a loud speaker, microphone or the like.

Diaphragms for use in electro-acoustic transducers such as a speaker or a microphone generally must satisfy the following requirements:

- (1) light in weight,
- (2) high rigidity (Young's modulus E) and moderate inner loss ( $\tan \delta$ )
- (3) a high ratio between the Young's modulus E and the density  $\rho$ , that is, specific modulus  $E/\rho$  or great sound propagation velocity  $\sqrt{E/\rho}$ .

The conventional materials for forming these diaphragms include:

- (a) those mainly composed of natural fibers such as plant fibers, animal fibers and mineral fiber,
- (b) the natural fibers as described above impregnated with thermosetting resin such as phenol resin or epoxy resin,
- (c) plastic sheet made of polypropylene, polyethylene terephthalate, etc.
- (d) metal member such as made of aluminum or titanium.

Among them, the diaphragms made of the natural fibers (a) as the main component can provide a flat frequency characteristic owing to their large inner loss  $\tan \delta$  but they are highly hygroscopic and cause fluctuations in the acoustic tone leading to degradation in the tone by way of aging.

Further, those natural fibers impregnated with a thermosetting resin such as phenol or epoxy resin as described in paragraph (b) above have a low inner loss  $\tan \delta$  and high density  $\rho$ . Accordingly, the plate thickness has to be reduced in order to decrease the weight of the diaphragm, which results in a defect of peak dip in the frequency characteristic. Further, although the diaphragm made of plastic sheets such as of polypropylene or polyethylene terephthalate as described in (c) above is excellent in water proofness, they are liable to cause deformation at a high temperature atmosphere of about 100° C. and require an increased cost.

Furthermore, although the diaphragm shaped by using metal members of aluminum or titanium as described in (d) above has a great Young's modulus E since the inner loss  $\tan \delta$  is small, it is difficult to damp the resonance at a higher frequency region, the ductility of the material is limited to worsen the workability and the cost is extremely expensive.

As described above, the materials (a)–(d) as described above, are not suitable as the material for forming the diaphragms for use in electro-acoustic transducers.

### SUMMARY OF THE INVENTION

This invention has been achieved in view of the foregoing problems and the object thereof is to provide a diaphragm for use in electro-acoustic transducers taking advantage of the natural fibers while compensating the drawbacks thereof, having a complete water proofness free from pin holes, with satisfactory workability, reduced in the cost, and capable of attaining flat frequency characteristic at high region, having large physical properties such as Young's modulus E, specific modulus elasticity  $E/\rho$  and sound propagation velocity

$\sqrt{E/\rho}$ . The features of this invention basically resides in a diaphragm for use in an electro-acoustic transducer comprising a laminate layer prepared by laminating a polyamide resin onto a diaphragm main body composed solely or mainly of natural fibers and a synthetic resin coating layer formed on the surface of the laminate layer.

### BRIEF DESCRIPTION OF THE DRAWINGS

These and other objects, features and the advantages of this invention will become clearer by the following descriptions made in conjunction with the appended drawings, wherein

FIG. 1 is a cross sectional view for one embodiment of a diaphragm for use in an electro-acoustic transducer according to this invention;

FIG. 2 is an enlarged cross sectional view for a portion within the circle A in FIG. 1;

FIG. 3 is a cross sectional view illustrating the step of manufacturing the embodiment shown above;

FIG. 4 is a cross sectional view for the state where a plastic film is laminated on the diaphragm main body; and

FIG. 5 is a characteristic chart for the respective sound pressure frequency characteristic for the diaphragm composed of polyethylene terephthalate and natural fiber according to this invention.

### DESCRIPTION OF THE EMBODIMENTS

This invention will now be described referring to several embodiments together with the manufacturing step in conjunction with the drawings.

FIG. 3 shows a device 1 as one embodiment used for practicing this invention. The device 1 comprises a lower die 2 and a upper die 3 mating to the lower die 2. The lower die 2 is formed at the inside thereof with a containing recess 1b in alignment with the shape of a desired diaphragm main body 4 and in communication with a suction port 2a, while the upper die 3 is formed at the inside thereof with an air supply recess 3b in communication with an air supply port 3a supplied with the pressurized gas such as a pressurized air. The diaphragm main body 4 is made, for example, of cone paper prepared from natural fibers by a paper making process or by spinning natural fibers in admixture with synthetic or semi-synthetic resin.

The diaphragm 4 is formed thereover with a laminate layer 5 which is made of water proofing and heat resistant plastic film such as of a thermoplastic polyamide resin. A synthetic resin coating layer 6 is formed on the surface of the laminate layer 5. The synthetic resin coating layer 6 is made, for example, of lacquer enamel paint or nitro-cellulose type having a high surface hardness.

For manufacturing the diaphragm 7, the diaphragm main body 4 is contained in the containing recess 2b of the lower die 2 at the first step and a polyamide resin film 5a as a water proofing and heat resistant thermoplastic material for forming the laminate layer 5 is disposed therabove between the lower die 2 and the upper die 3.

Then, the film 5a is heated to soften at a selected softening point as the second step.

Further, the upper die 3 is fitted to the lower die 2 while putting the film 5a between the upper die 3 and the lower die 2 in the third step. In this case, while the upper die 3 is usually lowered to the lower die 2, the

lower die 2 may be driven upwardly relative to the upper die 3.

Then, by sucking the air to evacuate in the containing recess 2b of the lower die 2 at the boundary of the film 5a through the suction port 2a by using the vacuum pump or the like at the third step 4 and supplying the pressurized air to the inside of the upper die 3 through the pressurizing port 3a at the boundary of the film 5a by using a compressor or the like. The film 5a softened by heating is deformed to form a laminate film 5 on the upper surface of the diaphragm main body 4.

Then, the synthetic resin coating layer 6 is formed on the surface of the laminate layer 5 as the fifth step to manufacture the diaphragm 7.

#### EXAMPLE 1

At first, a diaphragm main body 4 formed into a cone shape of about 30–400  $\mu\text{m}$  thickness by using pulp fibers of UKP20'SR as the natural fiber in the inside of the containing recess 2b of the lower die, while a polyamide resin film 5a of 20–50  $\mu\text{m}$  thickness is disposed thereinaabove between the upper die 3 and the lower die 2 and heated to soften at a temperature of about 150°C. for several seconds by a heater. Then, the inside of the containing recess 2b is evacuated by sucking through the suction port 2a of the lower die 2 with a suction pressure, for example, at about 20 cmHg, while pressurized air c is supplied to the inside of the pressurized supply port 3a of the upper die 3 under pressure by using a compressor to laminate a polyamide resin film 5a of about 20  $\mu\text{m}$  thickness to the upper surface of the diaphragm main body 4 thereby forming the laminate layer 5. Then, a synthetic layer coating layer 6 of about 100  $\mu\text{m}$  thickness made of nitrocellulose type lacquer enamel is formed by spray coating to the surface of the laminate layer 5 thus formed on the diaphragm main body 4 to manufacture a diaphragm 7.

In this example, the thickness of the polyamide resin 5a was chosen within a range from 20 to 50  $\mu\text{m}$ . If the film 5a of less than 20  $\mu\text{m}$  thickness is laminated to the diaphragm main body 4, it is not suitable in the case of the deep shape since the film 5a itself elongates. On the contrary, if a film 5a of a thickness greater than 50  $\mu\text{m}$  is laminated on the diaphragm main body 4, the weight of the diaphragm 7 is increased to worsen the sensitivity making it unsuitable to use.

#### EXAMPLE 2

At first, a diaphragm main body 4 formed into a cone shape of about 30–400  $\mu\text{m}$  thickness by using pulp fibers of UKP20'SR as the natural fiber in the inside of the containing recess 2b of the lower die, while a polyamide resin film 5a of 20–50  $\mu\text{m}$  thickness is disposed thereinaabove between the upper die 3 and the lower die 2 and heated to soften at a temperature of about 150°C. for several seconds by a heater. Then, the inside of the containing recess 2b is evacuated by sucking through the suction port 2a of the lower die 2 with a suction pressure, for example, at about 20 cmHg, while pressurized air c is supplied to the inside of the pressurized supply port 3a of the upper die 3 under pressure by using a compressor to laminate a polyamide resin film 5a of about 20  $\mu\text{m}$  thickness to the upper surface of the diaphragm main body 4 thereby form the laminate layer 5. Then, a synthetic layer coating layer 6 of about 100  $\mu\text{m}$  thickness made of a vinyl acetate resin is formed by spray coating to the surface of the laminate layer 5 to be

formed on the diaphragm main body 4 to manufacture a diaphragm 7.

Then physical properties such as the density  $\rho$ , Young's modulus E, inner loss  $\tan \delta$ , sonic propagation velocity  $\sqrt{E/\rho}$  and the like are compared for the diaphragm 7 for use in loud speaker in Examples 1 and 2 obtained in this way, a diaphragm shaped only from pulp fibers of UKP20'SR as the natural fiber not applied with lamination, conventional diaphragm shaped by laminating a polyamide resin of a 40  $\mu\text{m}$  thickness to the pulp fibers of UKP20'SR as the natural fiber not applied with lamination, conventional diaphragm shaped by laminating a polyamide resin of a 40  $\mu\text{m}$  thickness to the pulp fibers of UKP20'SR as the natural fiber and a conventional diaphragm for use in loud speaker shaped by using 100% by weight of polypropylene and 100% by weight of polyethylene terephthalate as the plastics. The results are shown in Table 1 below.

TABLE 1

| Diaphragm                                                                                                              | Physical property                     |                                                                          |                                               |                                                                                 |
|------------------------------------------------------------------------------------------------------------------------|---------------------------------------|--------------------------------------------------------------------------|-----------------------------------------------|---------------------------------------------------------------------------------|
|                                                                                                                        | Density<br>( $\text{g}/\text{cm}^3$ ) | Young's<br>modulus<br>$E \times 10^{10}$<br>( $\text{dyn}/\text{cm}^2$ ) | Inner<br>loss<br>$\tan \delta \times 10^{-2}$ | propa-<br>gation<br>velocity<br>$E/P \times 10^5$<br>( $\text{cm}/\text{sec}$ ) |
| UKP20'SR pulp<br>fibers                                                                                                | 0.60                                  | 2.0                                                                      | 5.0                                           | 1.8                                                                             |
| UKP20'SR pulp<br>fibers formed<br>with a lami-<br>nated film of<br>polyamide<br>resin of 40 $\mu\text{m}$<br>thickness | 0.63                                  | 2.1                                                                      | 5.5                                           | 1.8                                                                             |
| Polypropylene,<br>100% by weight                                                                                       | 0.90                                  | 1.8                                                                      | 9.0                                           | 1.4                                                                             |
| Polyethylene<br>terephthalate,<br>100% by weight                                                                       | 1.40                                  | 4.5                                                                      | 2.0                                           | 1.8                                                                             |
| Example 1                                                                                                              | 0.70                                  | 2.8                                                                      | 5.2                                           | 2.0                                                                             |
| Example 2                                                                                                              | 0.72                                  | 1.5                                                                      | 6.0                                           | 1.4                                                                             |

As apparent from the table 1 above, the density of the diaphragm in Examples 1 and 2 is slightly larger than the density of 0.60 ( $\text{g}/\text{cm}^3$ ) and 0.63 ( $\text{g}/\text{cm}^3$ ) in the diaphragms made of the UKP20'SR pulp fibers as the natural fiber and the diaphragm comprising the diaphragm main body made of UKP20'SR pulp fiber formed only with the polyamide resin laminate layer of 40  $\mu\text{m}$  thickness, but significantly lower than the density of 0.90 ( $\text{g}/\text{cm}^3$ ) and 1.40 ( $\text{g}/\text{cm}^3$ ) of the conventional diaphragm made of polypropylene or polyethylene terephthalate and, accordingly, greatly reduced in weight. Referring to the Young's modulus E, the diaphragm of Example 1 according to this invention has a large value of  $2.8 \times 10^{10}$  ( $\text{dyn}/\text{cm}^2$ ) as compared with the Young's modulus of  $1.8 \times 10^{10}$  ( $\text{dyn}/\text{cm}^2$ ) in the conventional diaphragm shaped from polypropylene. Further referring to the inner loss  $\tan \delta$ , while the inner loss  $\tan \delta$  of the conventional diaphragm shaped from the polyethylene terephthalate is  $2.0 \times 10^{-2}$ , the inner loss is  $5.2 \times 10^{-2}$  and  $6.0 \times 10^{-2}$  in the diaphragm of Examples 1 or 2 according to this invention which is significantly greater. Further referring to the sound propagation velocity  $\sqrt{E/\rho}$ , it is  $2.0 \times 10^5$  ( $\text{cm}/\text{sec}$ ) in Example 1 and  $1.4 \times 10^5$  ( $\text{cm}/\text{sec}$ ) in Example 2. The sound propagating velocity is greater in Example 1 rather than any of the conventional products shown in Table 1 and the sound propagation velocity in Example

2 is as large as that of the conventional diaphragm shaped from polypropylene.

Furthermore, since the diaphragm according to this invention is manufactured by forming a laminate layer 5 made of a polyamide resin film 5a formed to the upper surface of the diaphragm main body 4 made of UKP20'SR pulp fibers as the natural fibers and further forming at the surface thereof with a synthetic resin coating layer made of nitrocellulose type lacquer enamel paint or vinyl acetate resin, pin holes are utterly eliminated to attain a satisfactory water proofness that cannot be obtained in the conventional diaphragm only made of natural fibers or those conventional diaphragms merely forming the polyamide resin laminate layer to the diaphragm main body 4 made of natural fibers, as well as the invented diaphragm is excellent in the surface gross and, further, exhibit heat resistance even at a high temperature of about 100°C.

Furthermore, the diaphragm 7 in the Example 1 according to this invention can attain a flat frequency characteristic A inherent to the diaphragm made of natural fibers when compared with the conventional frequency characteristics B of the diaphragm made of 100% polyethylene terephthalate as shown in the sound pressure frequency characteristics in FIG. 5.

Although explanation has been made in the Examples 1 and 2 for the case of laminating the thermoplastic film 5a to the upper surface of the diaphragm main body 4, heat resistant and water proof plastic film 5a can, of course, be laminated on the lower surface and/or the upper surface of the diaphragm main body 4 by disposing the film 5a below the diaphragm main body 4 and containing them into the containing recess 2b of the

lower die and by mating the upper die 3 relative to the lower die 2.

As described above, since the laminate layer is formed by laminating the polyamide resin to the diaphragm main body only or mainly composed of the natural fibers and further forming the synthetic resin coating layer to the surface of the laminate layer in this invention, it is suitable as the material for forming the diaphragm free from pin holes, exhibiting a satisfactory water proofness and not impairing the physical properties such as the sound propagation velocity  $\sqrt{E/\rho}$  inherent to the natural fibers all over the diaphragm. Furthermore, different from the conventional diaphragm shaped from the metal member, since the diaphragm can be manufactured merely by laminating the diaphragm main body within the die and, thereafter, forming the synthetic resin coating layer to the surface of the laminate layer, it can be fabricated with ease, facilitate the fabrication work, does not worsen the yield and reduces the cost.

What is claimed is:

1. A diaphragm for use in an electro-acoustic transducer comprising

a diaphragm body of fabric material, said fabric material including natural fibers;

a preformed polyamide resin film having a thickness of 20-50  $\mu\text{m}$ , said polyamide resin film laminated to said diaphragm body;

a synthetic resin layer coated upon said polyamide resin film, said synthetic resin layer being selected from the group consisting of nitrocellulose type lacquer enamel and vinyl acetate resin.

\* \* \* \* \*